

# UNITED STATES PATENT OFFICE.

ISRAEL TOWNSEND, OF PORTSMOUTH, VIRGINIA.

## PAINT.

SPECIFICATION forming part of Letters Patent No. 398,917, dated March 5, 1889.

Application filed June 4, 1888. Serial No. 276,039. (No specimens.)

*To all whom it may concern:*

Be it known that I, ISRAEL TOWNSEND, a resident of Portsmouth, in the county of Norfolk and State of Virginia, have invented certain new and useful Improvements in Paints; and I do hereby declare the following to be a full, clear, and exact description of the invention, such as will enable others skilled in the art to which it pertains to make and use the same.

My invention relates to an improvement in paints; and it consists in the peculiar compound hereinafter described and claimed.

I first prepare a vehicle as follows: To one gallon of strong milk of lime (made from fresh caustic lime) one-half pound of powdered alum is added. I then add one gallon of linseed-oil and one-half pound of litharge. These ingredients, on being well stirred, readily unite and make a thick emulsion. When ready to use the paint, I stir into the vehicle thus prepared two pounds of metallic brown, two pounds of dry cement, and two pounds of fine dry sand, a sufficient quantity of these materials being stirred into the vehicle to make a good thick paint; but care must be taken not to mix these ingredients with the vehicle until the paint is to be used.

After the priming coat of my improved compound has been applied the same is permitted to dry. The second coat is then applied, the paint being the same as before, but some-

what thicker. When the paint has dried, it will be found perfectly impervious to water and as hard as stone.

When the last coat has been applied and before it dries, it is preferable that fine sand should be sifted on it.

For ordinary purposes two coats of my improved paint will be sufficient; but for unusually-exposed situations three coats should be applied.

I do not desire to limit myself to the precise proportions of the ingredients as hereinbefore described, as it is evident that the same may be varied without departing from the spirit of my invention.

Having thus described my invention, I claim—

1. The vehicle for paint, consisting of milk of lime, alum, linseed-oil, and litharge, substantially in the proportions specified.

2. The paint composed of the milk of lime, alum, linseed-oil, and litharge mixed with metallic brown, dry cement, and sand, substantially in the proportions described.

In testimony whereof I have signed this specification in the presence of two subscribing witnesses.

ISRAEL TOWNSEND.

Witnesses:

BALDWIN L. HOGE,  
THOMAS G. MANN.